

Patented Oct. 24, 1922.

1,433,180

# UNITED STATES PATENT OFFICE.

ARCHIBALD H. COPLAN, OF OTTAWA, ONTARIO, CANADA.

## ALLOY.

No Drawing.

Application filed March 7, 1921. Serial No. 450,604.

To all whom it may concern:

Be it known that I, ARCHIBALD H. COPLAN, a citizen of the Dominion of Canada, residing at Ottawa, in the county of Carleton and Province of Ontario, Canada, have invented certain new and useful Improvements in Alloys, of which the following is a specification.

My invention relates to an alloy, and 10 provides a material which is particularly designed for use in grate bars.

The object of my invention is to provide an alloy having constituents of metals, one of which is used in certain percentages to 15 resist the heat radiated from the coal or other fuel being burnt on such grate bars.

A further object is to provide an alloy having constituents of metals, one of which is used in certain percentages to close the 20 grain of the alloy so tight as to prevent the taking in to the composition any sulphur or other weakening elements from the coal or other fuel.

A further object is to provide an alloy 25 having constituents of metals, one of which is used in certain percentages to prevent warping by the grain of the composition being closed against receiving therein sulphur or other weakening elements from the 30 coal or other fuel.

A further object is to provide an alloy having constituents of metals, one of which is used in certain percentages to prevent the 35 oxidizing of the grate bars, and, therefore, extending its life and usefulness.

A further object is to provide an alloy having constituents of metals, one of which is used in certain percentages to prevent cracking by contraction or expansion when 40 used in combustion chambers.

I appreciate that compositions of alloy have been made, using the same metals in different percentages, with different other metals, without some of the metals herein- 45 after mentioned or for a distinct and entirely different purpose. After considerable experimenting and testing, I have found that if the hereinafter mentioned metals are formed into an alloy, it will provide an alloy which will be most efficient in the making of grate bars.

The constituents forming my alloy are as follows: Chromium approximately 1%, nickel approximately 2%, manganese .60% 50 to .75%, carbon .10% to .50%, balance principally iron with a small trace of sul-

phur .05% and under, phosphorus .05% and under, and silicon .35% to .50%. The sulphur, phosphorus and silicon will vary slightly and are well known in general 60 foundry practice.

Under severe tests, I have found that grate bars made from this alloy have proven more efficient and have lasted much longer. Chromium in the percentages above stated 65 has been found to resist the heat radiated from the fuel and at the same time close up the grain of the alloy so tight as to prevent any sulphur or other weakening elements to be taken in from the coal or other 70 fuel. This prevents any warping of the grate bars on account of these undesirable elements being excluded.

The percentage of the nickel is found to fully prevent oxidizing of the grate bars 75 under excessive heat. In other alloys, it has been experienced that the oxidizing, owing to the improper percentage of nickel will cause oxidizing and thus prove most inefficient.

In other alloys, different percentages of carbon have been used, but for the particular purpose for which this alloy has been designed, the low amount is sufficient for the purpose for which it is designed, and if 80 a higher carbon was used, it would be detrimental. A low carbon, in combination with other constituents provides an alloy, in which the carbon prevents cracking when the grate bars are under contraction or ex- 90 pansion.

What I claim as new is:

1. An article, which in use is exposed to combustion conditions, composed of an alloy embodying chromium approximately 95 1%, nickel approximately 2%, manganese not less than .60%, carbon not less than .10%, and iron with sulphur and phosphorus in small quantities.

2. A grate bar formed of an alloy embodying chromium approximately 1%, nickel approximately 2%, manganese not less than .60%, carbon not less than .10%, iron with sulphur and phosphorus in small quantities, and silicon not less than .35%. 100 105

In testimony whereof I affix my signature in the presence of two witnesses.

ARCHIBALD H. COPLAN.

Witnesses:

M. McMillan,  
M. Pendleton.